

May 8, 1928.

1,669,023

W. RUNGE

CARBONIZATION OF COAL

Filed Nov. 6, 1924



## UNITED STATES PATENT OFFICE.

WALTER RUNGE, OF EAST ORANGE, NEW JERSEY, ASSIGNOR, BY MESNE ASSIGNMENTS, TO INTERNATIONAL COAL CARBONIZATION COMPANY, A CORPORATION OF DELAWARE.

## CARBONIZATION OF COAL.

Application filed November 6, 1924. Serial No. 748,037.

The invention relates to the carbonization, distillation and/or gasification of coal and/or analogous materials and therefore the word "coal" as used herein is to be broadly construed as covering or including what is commonly known as coal and/or also all materials analogous thereto.

The invention has numerous aspects or objects, as will hereinafter clearly appear, among which there may be mentioned by way of illustration and not by way of limitation the following, and it will be noted that many others might be specifically referred to at this time.

15 Certain aspects pertain to the treating or pretreating of coal by a hot oxidizing medium under conditions whereby the coal loses its agglutinating properties or, in other words, the tendency for the particles to adhere and stick together, but under conditions whereby the coal loses only a small percentage of its hydrocarbon volatile content.

Another aspect relates to the treating or pretreating of coal—pulverized coal—by a hot gaseous medium while the fine particles of pulverized coal are suspended therein but under conditions whereby such particles retain substantially all the solid and hydrocarbon volatile constituents thereof prior to a subsequent processing of the coal for other purposes and while the coal is in finely divided form.

30 Other aspects relate to the pretreating of coal, preferably in pulverized form, under conditions to destroy the agglutinating properties or the tendency for the particles to stick together and the subsequent carbonization of the coal thus pretreated.

Another aspect relates to the precipitating of coal in finely divided form through a rising oxidizing atmosphere under conditions to overcome the tendency for the particles to adhere or stick together but under conditions whereby the coal loses only a small portion of its hydrocarbon volatile content, and the subsequent carbonizing or distilling of the coal thus pretreated while precipitating through a body of rising hot gases.

Further aspects relate to the treating of coal in finely divided form, preferably when dry, through the carbonizing action of a hot gaseous medium obtained by the withdrawal of gases from the process and reheated to the extent desired prior to reintroducing

them into the retort at a place where the reheated gases cause or effect the desired carbonization by upward movement of hot gases in direct contact with precipitating coal within the carbonizing zone.

A further object which may be enumerated involves the pretreating of pulverized coal by a hot medium, as an oxidizing medium within which the finely divided coal is suspended until it has been converted into a finely divided product, the pretreated particles of which do not tend to adhere to any appreciable extent but which retain practically all of the hydrocarbon volatile content, and the subsequent carbonization, distillation and/or gasification of the coal thus pretreated while the coal is suspended in a gaseous medium hotter than that of the pretreating gaseous medium.

It will be manifest that many other aspects or objects could be enumerated but it is not believed any further exemplification of the objects is necessary or advisable.

The drawing accompanying this specification and which constitutes a part thereof illustrates somewhat diagrammatically an apparatus within or by which the invention may be realized.

According to the sole figure thereof coal from storage or a crusher 1 is conveyed to a receiving hopper 2, passed to a drier 3, thence to a second receiving hopper 4 from which it passes to a pulverizer 5, thence to a third receiving hopper or storage bin 6 within which hopper dry pulverized coal is stored and from which it is withdrawn as desired.

*Pretreating retort.*

From the hopper or storage bin 6 the dry pulverized or finely divided coal is fed or showered, as by suitable means 7, into the upper portion of an unobstructed vertically extending treating or pretreating zone 8 within a retort or pretreating or preheating chamber 9. The construction of the feeding means 7 is such as to supply coal for treatment to the interior of the retort preferably under conditions whereby the coal will enter the retort without permitting the entrance thereto of any objectionable amount of cold air or the escape to the atmosphere of the hot gaseous medium from within the retort. The coal thus fed, which is manifestly in the form of fine particles, gravi-

tates but with a retarded gravitation toward the bottom or receiving space 10 of the pretreating zone 8. In transit the coal or material under treatment is subjected to the action of an upwardly moving hot gaseous medium, preferably an oxidizing gaseous medium, to wit, air, and gradually becomes precipitated as a fine treated product in which the coal particles do not tend to stick or adhere together; in other words, in this pretreating zone the coal is subjected to the effect of the hot air under conditions whereby the coal loses its sticky or agglutinating properties but under conditions whereby the coal loses only a small percentage of its hydrocarbon volatile content and thus the coal retains substantially or practically all the solid and hydrocarbon volatile content it originally possessed. From the bottom of the retort 9 or the receiving space 10 the treated, or pretreated coal as one may call it, is withdrawn as desired, preferably under conditions so as not to permit the entrance to the interior of the retort of objectionable cold air or the escape from the bottom of the retort of the hot gaseous medium therein. The means for permitting this withdrawal is indicated by 11 as a pair of sliding gates. The heat for maintaining the pretreating process is supplied at the bottom of the treating or pretreating zone 8; the gaseous treating medium with any gases entrained therein as a result of the pretreating process passes from the interior of the retort as through offtake piping 12. The pretreated product is conveyed in any suitable manner as through a closed conveyor 13 to a hopper 14 leading to a second feeding means 15.

#### Carbonizing retort.

The feeding means 15 is constructed so as to feed or shower the pretreated coal—which is in finely divided form which preferably still retains a substantial part of its heat and which may still be referred to as pulverized coal although it has been treated—into the upper portion of an unobstructed vertically extending carbonizing or distilling zone 16 within a retort or carbonizing chamber 17. The construction of the feeding means 15 is such as to supply the coal for treatment to the interior of the retort under conditions whereby the coal will enter the retort without permitting the entrance of any objectionable amount of air or the escape to the atmosphere of the gases from within the retort. The coal thus fed or showered—which is still in the form of fine particles—gravities downwardly in cloud-like form but with a retarded gravitation toward the bottom or receiving space 18 of the carbonizing zone 16. In transit the coal or material under treatment is distilled, carbonized and/or gasified by and while in suspension in upwardly moving hot gases and gradually be-

come precipitated as a fine carbonized residue—either a partially carbonized residue or a completely carbonized residue as desired—upon the parts of the structure defining the bottom of the receiving space 18. From the bottom of the retort or carbonizing chamber 17 or the receiving space 18 the carbonized residue is withdrawn as desired without permitting the entrance of objectionable air to the interior of the retort or without permitting the objectionable escape of gases to the atmosphere. The means for permitting this withdrawal is indicated by 19 as a sliding gate and by 20 as a screw conveyor. The heat for maintaining the carbonizing process is supplied at the bottom of the carbonizing or distilling zone 16, as will hereinafter more clearly appear. The gases of, or resulting from, the carbonizing or distilling process pass from the carbonizing zone; or, in other words, from the interior of the retort as through offtake piping 21 to any suitable gas purifying apparatus indicated as at 22; thence to holder 23 from which it is drawn as desired through pipe 24 and valve controlled pipes 25 and 26, the latter of which leads to a burner 27 for supplying heat to a heat interchanging device 28.

#### Heating systems for the retorts.

Each retort and its function has in a general way been described. The heating system for each will now be described. Reference has heretofore been made to the members 19 and 20 as controlling the withdrawal of the carbonized residue from the carbonizing zone 16. It will hereinafter appear that the process carried out in the carbonizing zone 16 is at a considerably higher temperature than that carried out in the pretreating zone 8. In other words, the carbonized residue from the zone 16 is comparatively hot and has a considerable residual heat which can be employed to good advantage in the pretreating zone 8. According to the construction shown the carbonized residue passes into a dry coke cooler 29 and the heat from the carbonized residue therein is indirectly transferred to air entering the coke cooler at 30 and leaving by pipe 31. If this air is sufficiently hot, that is has a temperature of approximately 800° F. (800 degrees Fahrenheit), then it is introduced directly into the bottom or lower portion of the retort 9 or, in other words, at the base or lower portion of the pretreating zone 8. If, however, the air thus supplied is not sufficiently hot enough, then it is supplied as through a heat interchanging device 32 which is heated in any suitable manner as by burner 33 supplied with the gas of the process and this heats the air entering at pipe 34, which after being heated passes through valve controlled pipe 35 into the pipe leading to the bottom of the retort. 130

The products of combustion from the burner 33 pass from the heat interchanging device 32 as by pipe 36.

If desired, the hot gaseous medium passing

- 5 to the retort 9 can be supplied not only to the pretreating zone 8 within the interior of the retort but it can be supplied to receiving space or spaces 37 defined in and by the walls of the retort whereby said walls 10 can be heated and maintained at the proper temperature desired.

Referring now to the heating system of the carbonizing retort, the burner 27 as previously indicated supplies heat to the heat interchanging device 28 and the products of combustion pass to the atmosphere by pipe 38. Gas for effecting the carbonizing process within the carbonizing zone 16 can by valve controlled pipe 25 be supplied to and 20 through the heat interchanging device 28 and when reheated to the extent desired it is supplied by means of pipe 39 to the lower portion of the carbonizing retort 17 or, in other words, at the base or lower portion 25 of the carbonizing zone 16. If desired, hot gas can also be supplied to the space or spaces 40 defined in and by the walls of the retort 17 whereby heat can, at will, thus be added or supplied for maintaining the desired temperature, or hot gas may even be introduced directly into the carbonizing zone 16, as through pipe 41.

According to the preferred mode of realizing or utilizing the invention the coal is subjected to a two stage process one of which stages is carried out in a preheating or pretreating retort and the second of which stages is carried out in the carbonizing retort and which are arranged and connected 40 so that the preheated material preferably passes to the carbonizing retort with a substantial amount of the heat therein; in other words, while the material is still in a relatively hot condition. It will be realized

these two retorts might in effect be embodied 45 in a single construction with a preheating section arranged above the carbonizing section.

Referring now to the process in detail, coal in finely divided form is conveyed or shown- 50 ered into the upper zone of the pretreating or preheating retort and it gravitates toward the bottom thereof. During its downward passage it encounters rising hot oxidizing gases, to wit, air. This air is previously 55 heated to approximately 800° F., enters the bottom of the pretreating retort at approximately said temperature, slowly flows toward and into the upper zones of the retort, and leaves the upper portion of the re- 60 tort at approximately 500° F.; in other words, the coal in its downward or gravitational passage is subjected to the retarding action and effect of the upwardly flowing gases—air—having an average temperature 65 of approximately 650° F. The retardation of the precipitation of the coal by the upward flow of the air is such that the coal particles are held in suspension approximately 30 seconds or, in other words, long enough 70 for the coal to attain a temperature of approximately 600° F. to 700° F. by the time it is precipitated at the bottom of the retort and the heat is sufficient to effect a removal of substantially all of the moisture and only 75 a small portion of the hydrocarbon volatile materials in the coal, and to cause the coal to lose practically all of its agglutinating or sticking together qualities. It will, therefore, be seen that the coal thus precipitated 80 falls as fine particles slightly enlarged above the size in which it was originally fed or showered because of the pretreatment and such oxidizing as is encountered within the retort. A specific example of coal thus treated in such a preheating or pretreating retort is typified as follows.

Coal having the following analysis—

|                      | Per cent. |
|----------------------|-----------|
| Moisture-----        | 1.5       |
| Volatile matter----- | 34        |
| (hydrocarbons)       |           |
| Fixed carbon-----    | 57.5      |
| Ash-----             | 7         |

This coal is sometimes referred to as high volatile coal.

and having a fineness indicated by the following:

|        |                                  |
|--------|----------------------------------|
| 59%    | passed through a 200 mesh screen |
| 85% "  | " 100 " "                        |
| 100% " | " 40 " "                         |

(A wire screen having 40,000 openings per square inch).

has been fed into a preheating retort having a treating zone of approximately 30 feet in height. The air for treating the coal was introduced at a temperature of approximately 800° F., caused to pass upwardly through 59 and in contact with the gravitating coal un-

til the air left the retort at approximately 500° F. and conveyed heat to the coal so that the coal has when precipitated a temperature of approximately between 600° F. and 700° 100 F. or, in other words, was subjected to the oxidizing and heating action of the air at

an average temperature of 650° F. The particles thus treated had an actual slight increase in size, as shown by the following,

38% passed through a 200 mesh screen  
 62% " " 100 " "  
 94% " " 40 " "  
 100% " " 20 " "  
 and had the following analysis:

|                 | Per cent. |
|-----------------|-----------|
| Moisture        | 0         |
| Volatile matter | 27        |
| Fixed carbon    | 65        |
| Ash             | 8         |

15 While the above indicates the type of treatment which may be carried out in this preheating chamber, it will be noted that the treatment and the resultant product will depend to a large extent upon the characteristics of the coal and of the thermal and chemical effects desired as a result of the pre-treatment.

16 The pretreated coal is preferably conveyed while still hot to the carbonizing retort. 25 There may be a slight loss of heat from the time of its accumulation, during its transfer, to the time of feeding into the carbonizing retort.

17 The coal fed into the upper zone of the carbonizing retort is showered so as to precipitate through an upwardly moving body or volume of hot gas or gases which is or are relied upon to perform the carbonizing operation within the retort. This carbonizing retort may be, for example, 50 feet high and of such diameter as may be determined and is supplied by hot gases introduced within the carbonizing zone under conditions whereby gas or gases from a zone having a temperature of approximately 1100° F. to 1500° F. 30 at the bottom rise or rises in contact with the precipitating coal and finally there leaves the retort at the upper portion thereof the gaseous products of the process at an approximate temperature of 550° F. to 850° F. In other words, the gravitating particles are subjected to a hot gaseous medium having average temperatures approximating between 825° F. and 1175° F. or an average of 35 this, to wit 1000° F. In a vacuum it would take roughly between one and two seconds for the coal particles to drop through a space of 30 feet to 50 feet. The rising current of gaseous medium in the carbonizing retort retards the fall of the particles being treated so 40 that in effect they are suspended in the gaseous medium approximately thirty seconds—sometimes more, sometimes less. This allows sufficient time with particles of the size indicated to become sufficiently heated so as to devolatilize the particles to a substantial extent. Practice has shown that by withdrawing coal of the character indicated, as 45 the result of the preheating operation when subjected in a carbonizing retort of the

height indicated and to gaseous mediums of the temperatures indicated there is produced a partially distilled residue having the following characteristics. Approximate analysis:

|                 | Per cent. |
|-----------------|-----------|
| Moisture        | 0         |
| Volatile matter | 12        |
| Fixed carbon    | 78        |
| Ash             | 10        |

75 and having a fineness indicated by the following—

|                                     | Per cent. |
|-------------------------------------|-----------|
| 7% passed through a 200 mesh screen | 80        |
| 21% " " 100 " "                     | 80        |
| 70% " " 40 " "                      | 80        |
| 100% " " 10 " "                     | 80        |

85 The residue from this carbonizing process was not agglutinated during the carbonizing process; nor did it assume a sticky condition when precipitated. In fact the same material was of a character which, if subjected to a carbonization direct from its raw state to the desired degree of devolatilization, would have developed objectionable agglutinating characteristics which would have followed to the end and been found as lumps or agglomerations in the resultant products. The 90 preheating treatment previously described was simply to and actually did overcome 95 said objectionable feature.

100 The heat for carrying out the carbonizing treatment may be realized by supplying a controlled and limited amount of air into the lower zone of the carbonizing retort so as to support a partial combustion in said lower zone; for example, according to the process of my companion application identified as Case B, to wit, U. S. application Serial Number 748,038 filed November 6, 1924; or, it may be supplied as is clear from the drawing hereof by means of reheated, clean gas obtained by withdrawing gas from the top of the retort, cooling and removing any byproducts and otherwise cleaning; reheating a portion of the withdrawn gases by means of a heat interchanger and introducing the reheated gases into the lower zone of the retort at temperatures approximating between 1100° F. and 1500° F. and continuing the operation while withdrawing surplus gas and conducting it to the holder or otherwise using the same as may be found desirable. It will be noted that in event the hot 110 gases for performing or affecting the carbonization process—be they the hot products resulting from combustion or the reheated gases obtained from the process—are gases which are substantially chemically inert with respect to the coal undergoing carbonization. 115 Some of the gas may be used if desired for preheating the air used in the pretreating process. A fair estimate of the solid and gaseous products made and used in the process is indicated somewhat as follows: 120

70

75

85

90

95

100

105

110

115

120

125

130

For each ton of material fed into the upper portion of the carbonizing retort and subjected to carbonization by gaseous medium having an average temperature of upwardly 1000° F. there are produced from the coal approximately 3500 cubic feet of gas having a B. t. u. value of 800 B. t. u. per cubic foot and there are used in the process for preheating purposes approximately 1500 cubic feet of gas having a B. t. u. value of 800 B. t. u. per cubic foot, leaving a surplus of 2000 cubic feet of the same type of gas for each ton of coal treated. This is in addition to condensable gases removed in the form of liquids.

According to the apparatus shown the gas that is used for performing the carbonizing process is, as above indicated, first subjected to suitable purification apparatus, indicated at 22, in which it is freed of the oil, tar, etc., as is customary in gas practice. The cool, clean gases are divided. Some go to the holder or other place of use while some are used in the carbonizing retort after passing through a heat interchanger 28 which superheats them to the desired temperature of approximately 1100° F. to 1500° F. Within the carbonizing retort the superheated gas performs the carbonizing process previously described.

In the form of apparatus shown, it is possible to pass air through the dry coke cooler or heat interchanger 29 at the bottom of the carbonizing retort so that the air absorbs some of the heat from the coke and the air thus to a certain extent is preheated and passes directly to the pretreating chamber 9; or, it may be passed into an air heater or heat interchanger 32 for bringing the air up to the desired temperature of approximately 800° F. and from this source the air is supplied to the interior of the pretreating retort where it performs the process previously described.

45 What I claim is:

1. A method comprising subjecting coal in finely divided form to carbonization by feeding it into the upper portion of a carbonizing zone, within which zone the coal precipitates counter to and in direct contact with an upwardly moving gaseous medium that delays the settling of the precipitating coal and which is hot enough to carbonize to the desired extent the precipitating coal, and collecting the coal as partially carbonized residue, said hot gaseous medium being created and maintained by and from gases withdrawn from the process and thereafter cooled and purified and some of which are thereafter reheated to between 1150° F. and 1500° F. and returned in reheated condition into the lower portion of the carbonizing zone to create the upwardly moving gaseous medium.

60 2. The carbonizing of coal by the method

which comprises feeding dry finely divided coal into the top of a carbonizing chamber and causing a delayed precipitation of the finely divided coal by a counter current of hot gases caused by the introduction to the bottom of the carbonizing chamber of gases of the process indirectly reheated to between 1150° F. and 1500° F., withdrawing from the top of the carbonizing chamber gases resulting from the process at approximately 550° F. to 850° F., and collecting the partially carbonized residue resulting from this process.

3. The carbonizing of coal by feeding finely divided coal into the top of a defined carbonizing zone and effecting a delayed precipitation of the finely divided coal by a counter current of hot gases caused by the introducing at the base of the carbonizing zone of gases of the process reheated to upwardly of approximately 1150° F., withdrawing from the top of the retort of gases resulting from the process, cooling and purifying said withdrawn gases, reheating some of said cooled purified gases and thereafter returning the reheated gases to the carbonizing zone for effecting the carbonizing operation, and collecting as partially carbonized coal the precipitated residue resulting from the process.

4. The process of carbonizing coal comprising showering pulverized coal from within the upper portion of a confined carbonizing zone and causing a delayed precipitation of the finely divided coal by hot gases moving upwardly because of the introduction to the bottom of the carbonizing zone of gases withdrawn from the process and indirectly heated prior to such introduction, withdrawing from the top of the retort gases resulting from the process, indirectly reheating to between 1150° F. to 1500° F. some of the withdrawn gases and reintroducing them into the bottom of the carbonizing zone for the purpose outlined, collecting the partially carbonized residue in a receiving space below the carbonizing zone and into which space the partially carbonized residue gravitates from the carbonizing zone, and withdrawing precipitated partially carbonized residue from said receiving space.

5. The method which comprises subjecting coal in finely divided form to carbonization by flowing hot gases within which the coal is suspended while being carbonized, withdrawing gases of the process, indirectly reheating some of the withdrawn gases upwardly of 1150° F. but not substantially above 1500° F. and returning said reheated gases to the process for maintaining the flowing hot gases necessary for the process, and collecting the resulting carbonized residue.

6. The process comprising subjecting

5 finely divided coal having agglutinating properties in suspension to the effects of a hot oxidizing gaseous medium for destroying the agglutinating properties of the coal and until the agglutinating properties have 10 been destroyed but under conditions whereby the coal retains substantially all the solid and hydrocarbon content of the coal and whereby the coal loses at the most only a small percentage of its hydrocarbon volatile content, and thereafter carbonizing the still 15 finely divided coal while in suspension in hot gases which are chemically inert with respect to the coal.

15 7. The method comprising preliminarily subjecting pulverized coal having agglutinating properties to hot air by suspending the coal in the hot air until the coal loses its agglutinating properties and loses of its 20 volatile content only a small percentage thereof and so that the coal retains its finely divided state, and finally subjecting the coal to carbonization in hot gases chemically inert with respect to the coal and under conditions to leave a finely divided carbonized residue.

25 8. The treating of coal by the process comprising suspending pulverized coal having agglutinating characteristics in and subjecting it to heated air until the coal particles have attained a temperature of approximately 650° F. and have lost their agglutinating characteristics and thereafter in a non-oxidizing atmosphere subjecting the coal 30 to carbonization.

35 9. The method comprising in one retort subjecting finely divided coal having agglutinating properties to hot oxidizing gases until the coal loses its agglutinating properties but under conditions to remove only a small percentage of the hydrocarbon volatile content of the coal and thereafter in another retort subjecting the coal while 40 finely divided and in suspension in hot gases chemically inert with respect to the coal to carbonization so as to distill off a substantial percentage of the hydrocarbon volatile content of the coal but under conditions to leave a finely divided carbonized residue.

45 10. The method comprising feeding pulverized coal having agglutinating properties into a pretreating zone and subjecting the pulverized coal in and to hot gases until the coal has lost its agglutinating properties and 50 under temperature conditions so that the coal loses only a little of its hydrocarbon volatile content, and thereafter transferring the coal to a carbonizing zone and therein suspending and subjecting the coal in and to 55 hotter gases and under conditions so that much of its hydrocarbon volatile content is distilled off and so as to leave the solid carbonized residue in finely divided form.

60 11. The treating of coal by the method comprising feeding coal which is in finely di-

70 vided form and which has agglutinating properties into a pretreating chamber and therein subjecting the finely divided coal to the action of a hot oxidizing medium while the coal remains suspended in the hot oxidizing medium until the coal has lost its agglutinating or adhesive properties and thereafter in a carbonizing chamber or retort subjecting the coal thus treated and while still in finely divided form to a carbonizing ac- 75

76 12. A process which comprises subjecting finely divided coal having agglutinating properties and having a high hydrocarbon volatile content and which is in suspension in a hot oxidizing atmosphere to the action thereof under conditions whereby the coal loses only a small portion of its volatile content but until it has lost its agglutinating properties, separately removing the coal thus pretreated on one hand and the gases for and resulting from the pretreating operation on the other, thereafter subjecting the coal thus treated but while still in finely divided condition to a carbonizing action of another hot gaseous medium which is chemically inert with respect to the coal with the coal in suspension therein under conditions whereby the coal thus treated loses a substantial portion of its volatile content and is converted into finely divided carbonized residue, and separately removing the resulting carbonizing coal residue on the one hand and the said last mentioned gaseous medium and the gases resulting from the carbonizing action on the other and in such manner that the last mentioned gases are not mingled with the gases for or of the pretreating operation.

80 13. The method which comprises suspending and subjecting pulverized coal having agglutinating properties to the action of hot air until the coal has lost its agglutinating properties but under conditions to leave substantially all of the hydrocarbon volatile content of the coal, causing the coal thus pretreated to pass to a carbonizing zone and therein suspending and subjecting the pretreated coal, while still in finely divided form to the action of rising hot gases chemically inert with respect to the coal and sufficiently hot to effect a desired carbonization 85 of the coal in suspension, collecting the gases of the carbonization process, and withdrawing the resulting finely divided carbonized residue precipitated from the carbonizing zone.

90 14. A method comprising subjecting dry pulverized coal having agglutinating properties to pretreatment by subjecting it to the action of hot gaseous mediums under conditions by which the coal loses its agglutinating properties but so as to leave in the pretreated coal substantially all of its original 95 hydrogen volatile content, thereafter passing the finely divided pretreated coal to the up-

- per portion of a carbonizing zone downwardly within which the coal thus fed precipitates counter to and in direct contact with an upwardly moving hot gaseous medium that is substantially chemically inert with respect to the coal and which delays the settling of the precipitating coal and which is hot enough to and does carbonize to the desired extent the coal while precipitating, and collecting the resulting coke residue. 10
15. The method which comprises subjecting pulverized coal having sticky characteristics that develop when heated by suspending the coal in a hot oxidizing medium to the action thereof under conditions to cause the coal to lose its tendency for the particles to adhere to each other, conducting the coal thus treated to a hot carbonizing zone and therein subjecting the coal to the action of a 15 gaseous medium sufficiently hot to effect a desired carbonization of the coal and within which the coal is suspended until the desired carbonization is realized, withdrawing the gases of the process, reheating some of the 20 withdrawn gases and returning the reheated gases to the interior of the carbonizing zone to provide the hot gaseous medium for maintaining the process, and withdrawing at will the carbonized residue resulting from the 25 process. 30
16. The method comprising precipitating and subjecting pulverized coal having agglutinating properties into and to the action of hot air having an average temperature of approximately 650° F. under conditions that the coal comes to a temperature of approximately 650° F. but under conditions whereby the coal while in contact with the air loses its agglutinating properties but 35 little of its volatile content, thereafter subjecting the coal to carbonization by a low temperature distillation process, withdrawing the gases of the low temperature distillation from the distillation zone, and also 40 withdrawing the carbonized residue resulting from the low temperature distillation. 45
17. The method comprising feeding pulverized coal having agglutinating properties and with a substantial hydrocarbon volatile content into the top of a pretreating chamber, and subjecting it while precipitating to a counter flow of a hot gaseous medium maintained by continuously feeding air into the bottom of the pretreating chamber at a 50 temperature of approximately 800° F., continuously withdrawing the gaseous medium from the top of the pretreating chamber at a temperature of 500° F. and subjecting the pretreated coal to carbonization. 55
- 60 18. The treating of coal by the method which comprises precipitating pulverized coal having agglutinating characteristics through rising hot air having temperatures approximately between 500° F. and 800° F. 65 and until the coal has a temperature of ap-
- proximately 650° F., thereafter causing precipitation of the coal while still in finely divided condition through an upwardly flowing hot gaseous medium so as to effect carbonization while in suspension in the gaseous medium, said gaseous medium having final temperatures between 500° F. and 800° F. and initial temperatures of between 1150° F. and 1500° F., and collecting the resulting residue in finely divided form. 70
19. The method which comprises suspending pulverized coal having agglutinating properties in hot air and subjecting the suspended coal to the action of the hot air until the pulverized coal has lost its agglutinating properties but under conditions that the coal loses only a small percentage of its hydrocarbon volatile content, conveying the coal thus pretreated and which is still finely divided and while still hot to a carbonizing zone and therein suspending the pretreated coal in a gaseous medium which is hotter than the air, and subjecting the suspended pretreated coal to the action of the hotter gaseous medium until a substantial percentage of the hydrocarbon volatile content of the coal is distilled off, withdrawing gases from the carbonizing zone, and withdrawing the resulting finely divided carbonized residue. 75
20. A method comprising feeding dry pulverized coal having agglutinating properties into the top of a pretreating retort within which the coal thus fed precipitates counter to upwardly moving hot air and permits and causes delayed settling of the precipitating coal particles until the coal has become heated to approximately 650° F. and has lost the properties whereby the particles adhere or stick together, causing the finely divided preheated coal which still retains substantially all of its original hydrocarbon volatile content to pass the top of a carbonizing retort within which the coal thus fed precipitates counter to an upwardly moving hot gaseous medium that permits and causes delayed settling of the precipitating pretreated coal particles and which hot gaseous medium is hot enough to carbonize to the desired extent the precipitating pretreated coal, and collecting the precipitated carbonized residue. 80
21. The method comprising feeding pulverized coal having agglutinating properties into the top of a confined pretreating zone 100 and subjecting it to a counter current of a hot gaseous medium maintained by feeding air into the bottom of the pretreating zone at a temperature of approximately 800° F. and withdrawing the gaseous medium from the top of the pretreating zone at a temperature of 500° F., thereafter subjecting the pretreated coal in finely divided form and while precipitating through a confined carbonizing zone to a counter current of up- 105
- 110
- 115
- 120
- 125
- 130

wardly flowing hot gaseous medium having a temperature at the bottom of the carbonizing zone of between 1150° F. and 1500° F., withdrawing gases of the process from the 5 top of the carbonizing zone at temperatures between 550° F. and 850° F. and collecting the resulting carbonized residue.

22. The process of treating coal with high volatile content and having agglutinating 10 characteristics which comprises pulverizing the coal until at least 50% will pass through a 200 mesh screen and so that all of it will pass through a 30 mesh screen, showering the coal through a hot zone while subject- 15 ing it to a rising current of hot gaseous me-

dium having an average temperature of 650° F. and under conditions whereby the coal will remain suspended approximately 30 seconds, and showering the solid product through a hot zone while subjecting it to a 20 rising current of hot gases having an average temperature of approximately 1050° F. and under conditions whereby the coal will remain suspended in the hot gases approximately 30 seconds, and collecting the finely 25 divided residue resulting from the process.

In witness whereof I have hereunto signed my name.

WALTER RUNGE.